

# UNITED STATES PATENT OFFICE.

EDWIN CUNO KAYSER, OF CINCINNATI, OHIO, ASSIGNOR TO THE PROCTER AND GAMBLE COMPANY, OF CINCINNATI, OHIO, A CORPORATION OF OHIO.

## PROCESS FOR RENDERING FINELY-DIVIDED CATALYTIC NICKEL NON-PYROPHORIC AND STABLE.

1,001,279.

Specification of Letters Patent. Patented Aug. 22, 1911.

No Drawing.

Application filed December 27, 1909. Serial No. 535,143.

*To all whom it may concern:*

Be it known that I, EDWIN CUNO KAYSER, a subject of the King of Great Britain, and now residing at the city of Cincinnati, in the county of Hamilton and State of Ohio, have invented a certain new and useful Process for Rendering Finely-Divided Catalytic Nickel Non-Pyrophoric and Stable, of which the following is a full, clear, and exact description.

Finely divided nickel powder, such as is obtained by reducing a suitable nickel compound at elevated temperature in a current of hydrogen, and such as of late finds employment in various chemical processes as a so-called "catalyzer", possesses well known pyrophoric tendencies. Even when the material has, at the end of the reduction-period, been permitted to thoroughly cool in an atmosphere of hydrogen, on withdrawal from the apparatus and consequent exposure to air, it is liable to spontaneous ignition or at least to a rapid rise in temperature, indicating fatal oxidation. Powders with such tendencies are difficult to handle even on the smallest scale, and it is readily understood that they do not meet industrial and commercial requirements. The same strictures in a measure apply to such preparations, as represent finely divided nickel, diffused among or deposited upon some inert material.

The object of this invention is to greatly diminish or entirely suppress these pyrophoric tendencies without interference with catalytic energy, and the manner and method for bringing about this result is as follows:

Nickel oxide, hydrate, or their equivalents, or inert materials, impregnated or coated with these compounds, are heated in a current of hydrogen in a suitable apparatus and in such manner and under such conditions, as are known to effect reduction and to yield catalytic metal, a temperature of five hundred to six hundred degrees centigrade being preferably maintained. As soon as reduction is judged complete, which will be the case when no more steam is evolved, a brisk current of carbonic acid is turned into the apparatus, meantime maintaining the former temperature. This treatment is continued for a considerable

time, varying from one to several hours, according to the volume of the gas current, 55 construction and size of apparatus, and weight and nature of charge; it must in no case be interrupted until the escaping gas proves no longer inflammable, and it shall be continued beyond that period for such 60 time, as actual experiences prove desirable in each particular case. At the termination of such period the apparatus and the material contained therein are cooled more or less rapidly, according to provisions 65 made toward that object, a moderate current of carbonic acid being maintained continuously through the apparatus to prevent the ingress of air.

When the apparatus and its contents have 70 attained normal temperature, the gas current may be discontinued, but the apparatus remains closed and the charge is not withdrawn for several hours, such period of quiescence assisting toward the desired end. 75

If the manipulation described has been carried out with proper care and with due consideration of existing circumstances, the metallic powder or metalliferous material thus prepared will remain perfectly cold on 80 exposure to air and may thus be exposed for days without thereby losing any of its initial catalytic energy. Unsuitable deviation from the lines laid down makes itself perceptible by a corresponding deviation 85 from the desired result.

What I claim as new, and of my invention and desire to secure by Letters Patent, is:—

1. The method of rendering finely divided nickel non-pyrophoric and stable in the air, 90 which consists in subjecting it, at elevated temperature, to the prolonged action of carbonic acid gas and subsequently cooling it in an atmosphere of carbonic acid gas.

2. The method of producing finely divided 95 nickel, non-pyrophoric and stable in air, which consists in reducing a nickel compound with hydrogen at a high temperature and thereafter, at elevated temperature, subjecting the powder to the action of carbonic 100 acid gas, and subsequently cooling in an atmosphere of carbonic acid gas.

3. The method of producing finely divided nickel, non-pyrophoric and stable in the air, 105 which consists in reducing a nickel compound, at elevated temperature, in a current

2  
of hydrogen and thereafter, while maintaining the temperature, submitting the resulting metallic powder to a current of carbonic acid gas and finally cooling in an atmosphere of carbonic acid gas.

4. The method of rendering finely divided nickel, diffused through or deposited upon an inert refractory material, non-pyrophoric and stable in the air, which method consists in subjecting such material, at elevated temperature, to the prolonged action of carbonic acid gas and subsequently cooling it in an atmosphere of carbonic acid gas.

5. The method of producing finely divided nickel, diffused through or deposited upon an inert refractory material, non-pyrophoric and stable in the air, which method consists in submitting such a material, impregnated or coated with a nickel compound, at elevated temperature, successively to a current of hydrogen and of carbonic acid gas and finally cooling it in an atmosphere of carbonic acid gas.

6. Finely divided nickel, rendered non-pyrophoric and stable in the air by the prolonged action thereon of carbonic acid gas at elevated temperature and by subsequent

cooling in an atmosphere of carbonic acid gas.

7. Non-pyrophoric, stable, finely divided nickel, produced by submitting a nickel compound at elevated temperature successively to a current of hydrogen and of carbonic acid gas and finally cooling in an atmosphere of carbonic acid gas.

8. Non-pyrophoric, stable, finely divided nickel, diffused through or deposited upon an indifferent material, submitted, at elevated temperature, to the action of carbonic acid gas and finally cooled in an atmosphere of carbonic acid gas.

9. Non-pyrophoric, stable, finely divided nickel, diffused through or deposited upon an indifferent material, obtained by submitting such material, coated or impregnated with a nickel compound, at elevated temperature, to the successive action of hydrogen and of carbonic acid gas and finally cooling in an atmosphere of carbonic acid gas.

EDWIN CUNO KAYSER.

Witnesses:

EARL W. GRIFFIN,  
MARSTON ALLEN.